

# UNITED STATES PATENT OFFICE.

OSCAR WARREN PICKERING, OF SPRINGFIELD, MASSACHUSETTS, ASSIGNOR TO  
PICKERING PAINT & PIGMENT COMPANY, A CORPORATION OF WEST VIR-  
GINIA.

## PAINT AND PIGMENT.

1,181,588.

Patented May 2, 1916.

No Drawing.

Application filed August 4, 1915. Serial No. 43,615.

To all whom it may concern:

Be it known that I, OSCAR WARREN PICK-  
ERING, a citizen of the United States, re-  
siding at Springfield, in the county of  
5 Hampden and State of Massachusetts, have  
invented certain new and useful Improve-  
ments in Paint and Pigment, of which the  
following is a specification.

This invention relates to a new pigment  
10 and paint thereof and has for some of its  
objects the production of a pigment or paint  
which will have greater spreading power,  
less disintegrating or decomposing character  
when exposed to ingredients of or associated  
15 with the atmosphere, more permanency or  
stability when exposed to light, and less  
specific gravity, whereby the settling out  
from the paint vehicle is prevented, and  
which will be more readily miscible with  
20 oils or other vehicles than such substances as  
"white lead," contain less lead and pro-  
duces greater and better results, and it con-  
tains a compound or composition of metal  
aluminate and metal hydroxid such as a  
25 compound or composition of lead with alu-  
minium and oxygen in the form of lead  
aluminate or its equivalent combined or as-  
sociated with a hydroxid, such as lead  
hydroxid, and the same associated with a  
30 vehicle such as a drying oil of the linseed  
type and in some cases with a diluent of  
drying nature such as turpentine, in the  
form of paint or similar commodity.

When ordinary "white lead" is employed in  
35 or as a paint associated with such vehicles as  
linseed oil and turpentine the gravity of  
the lead compound or composition which  
comprises a lead carbonate and hydroxid  
(hydrate) in proportion of approximately  
40 two parts of the former to one part of the  
latter, or chemically  $2\text{PbCO}_3 - \text{Pb}(\text{OH})_2$ , is  
such that it soon separates or settles out  
from mixed paint and is hard to remix again  
45 to a uniform consistency. The lead com-  
pound or composition when exposed to the  
atmosphere is readily attacked and decom-  
posed by sulfur therein and turned black  
and it is to obviate these and other difficul-  
ties that the present invention is devised.

50 The lead aluminate which is preferred  
in conjunction with the metal or lead hy-  
droxid is the normal aluminate and the pig-  
ment is produced by the action of lead ace-

tate on sodium aluminate and sodium hy-  
droxid (caustic soda) thus:—



The sodium acetate is washed out of the  
lead aluminate and lead hydroxid precipi-  
tate and the acetic acid recovered by treat-  
ment with a stronger acid such as sulfuric. 60  
The lead aluminate and lead hydroxid thus  
produced is thoroughly washed and dried,  
yielding a white product of superior mixing  
qualities with oils and producing a paint 65  
which readily spreads and presents a body  
covering of great light diffusive quality.

It will be noted that the lead aluminate  
and lead hydroxid contains aluminium oxid  
in place of carbon dioxide of the ordinary 70  
"white lead" which is more permanent and  
less affected by decomposing ingredients of  
the atmosphere and it more readily assimili-  
ates with oils or other paint vehicles and  
especially with drying oils, such as linseed, 75  
tung, and the like, or the same associated  
with driers such as turpentine.

Instead of a pigment composed of lead  
aluminate and lead hydroxid, the lead alum-  
inate may be associated with any other metal 80  
hydroxid or hydrate, such as aluminium  
hydroxid, zinc hydroxid, etc., corresponding  
to "white lead" except that the lead car-  
bonate is substituted by lead aluminate and  
the lead hydroxid by another metal hydroxid 85  
or like lead hydroxid thus:—

White lead.  $2\text{PbCO}_3 - \text{Pb}(\text{OH})_2$ .

New pigment.  $2\text{PbAl}_2\text{O}_4 - \text{Pb}(\text{OH})_2$ .

Or with different metal hydroxid.  $2\text{PbAl}_2\text{O}_4 - \text{Al}_2(\text{OH})_6$ .

This compound or composition of lead  
aluminate and lead or other metal hydroxid  
or hydrate may be produced by acting on a  
mixture of sodium aluminate and sodium 95  
hydroxid or hydrate with lead acetate or  
lead acetate and a soluble compound of an-  
other metal compatible with lead acetate  
without decomposition such as aluminium  
acetate or zinc acetate, or a mixture of lead 100  
acetate and acetic acid in cases where alu-  
minium hydroxid is desired associated with  
the lead aluminate as shown in the third  
formula in which case sodium aluminate is  
employed without the sodium hydroxid  
(caustic soda).

The lead aluminate and lead or other

metal hydroxid are thrown down or precipitated from the aqueous solution of the compounds referred to in such an intimate state of division and admixture as to present the appearance of an actual chemical compound similar to the lead carbonate and lead hydroxid (hydrate) compound or composition of the so-called "white lead."

It will be noted that in the compound 10 comprising lead aluminate and lead or other metal hydroxid, the percentage of lead in the compound over that contained in white lead or lead carbonate thereof is reduced and the bulk of the paint increased by the 15 employment of the aluminate and the product is therefore much cheaper as to cost than white lead while at the same time it yields a product of greater superiority over the old form of lead carbonate and hydrate 20 both as to spreading power and resistance to atmospheric decomposition thereby rendering it more permanent in character.

It is obvious that the lead aluminate and lead or other metal hydroxid may be produced in any convenient manner other than 25 that described and that the pigment may be associated with any selective vehicle in producing the paint without departing from the spirit of the invention which broadly 30 comprises as a new pigment or paint a metal aluminate and metal hydroxid or its equivalent, or specifically lead aluminate and lead hydroxid or lead aluminate associated or combined with a metal of like or unlike 35 character in the form of a hydroxid or hydrate or specifically lead, aluminium, zinc, or other metal hydroxid or hydrate, or such compounds or compositions associated with a paint vehicle, such as a drying oil (linseed) or the same with a drier (turpentine).

The so-called "white lead" contains lead 45 compounds which are slightly soluble in water and produce a poisoning effect when employed, to the painter, the maker and the user, which is largely prevented if not entirely avoided in the making, employment and the use of the less soluble lead aluminate and metal hydroxid in place of the lead carbonate and lead hydroxid which is contained 50 in white lead.

In the manufacturing, shipping, and dispensing of mixed paints the lead aluminate and metal hydroxid pigment is of great utility, in that its lesser gravity than white lead maintains it in a mixed or suspended condition in the paint vehicle, thus avoiding the settling out of the pigment to a great extent and yielding a more uniformly mixed paint and maintained as such, which is of greater utility, durability, spreading power, and practical utility, than pigments and paints of mixed character employed hitherto.

As an example of the manner in which a 65 metal aluminate such as lead aluminate and a different metal hydroxid may be produced

reference is directed to the following chemical formula or equation which illustrates the formation of lead aluminate and aluminium hydroxid by the interaction of sodium aluminate and lead acetate and acetic acid:—



Any metal aluminate may be employed, such as copper, magnesium, chromium, iron, 75 mercury, nickel, calcium, or other metal aluminate, which aluminate may be simple, compound, complex or composite in nature and may be associated with like or unlike metal hydroxid in chemical combination or physical association without departing from the spirit of the invention and any other metal hydroxid may be substituted for the lead hydroxid in the lead aluminate compound or composition, such as aluminium, 80 zinc, or other metal hydroxid.

It is obvious that the metal of the aluminate may exist at any atomicity and the aluminate may comprise the normal, basic, or other variety, without departing from the 90 spirit of the invention.

Some of the preferable species of aluminate employed comprise, and in connection with the present invention with preferable 95 reference to cheapness and utility may be noted as, calcium aluminate, copper aluminate, and zinc aluminate, either *per se* or associated or combined with other substances, ingredients or vehicles.

The term or expression "paint" as employed herein is intended to imply and does 100 imply a pigment or dry paint as such or associated with a vehicle or carrier of any suitable kind, preferably of liquid character, capable of enabling the associated pigment or dry paint to be spread on a surface in a coating by means of a brush or its equivalent; the term or expression "vehicle" implies a pigment or dry paint carrier, preferably of fluid nature, which may consist of 105 or comprise any suitable character comprising one which may evaporate entirely, leaving the pigment or dry paint upon the surface or within the pores of the article to which it is applied, such as water, benzine, etc., or the same associated with a paint fixative, such as gum, resin, casein compounds, etc., or it may comprise an oil of any suitable kind such as a petroleum product, vegetable oil of drying or non-drying character, etc., so long as it acts to carry the pigment or dry paint and enhance the spreading thereof by action of a brush or its equivalent, or the oil and pigment may be associated with a suitable fixative or drier; and the term "drier" implies a substance or constituent of the oil or paint composition which is capable of fixing the oil or paint by transforming it into a gelatinous or non-fluid condition by acting as an oxygen car- 115 120 125 130

- rier to the oil forming a non-fluid oil oxygenated compound, such as linoxyn, or an oil setting or gelatinant, such as metal soap or oleates or resinates either directly employed or formed in the paint by interaction of the ingredients, such as the resin acids formed by oxidation of turpentine and their action on a pigment or dry paint metal compound constituent. For example, the drying or transforming of a fluid non-drying petroleum product or vegetable oil into a non-fluid or fixed gelatinous condition, as a pigment or dry paint vehicle or fixative may be accomplished by associating the pigment or dry paint, such as lead aluminate and non-drying vegetable oil, such as cottonseed oil, with turpentine which, when it is spread on a surface and exposed to oxygen of the air, results in the conversion of the turpentine into resin acid aldehydes, which united with the lead and aluminium content forming resinates, also the oil or propenyl or glycercyl oleate, reacts, with the lead aluminate forming lead glycerinate, lead and aluminium oleate and resin and aliphatic or oleic acid ethers, all of which products, resinates, oleates, glycerinates and ethers increase the viscosity, absorb, combine with, retain, or occlude the excess of oil and the pigment transforming the whole into a gelatinous or non-fluid and substantially dry condition, just as water is retained or dried by gelatin or glue, in this manner oils of ordinarily non-drying character may be employed as well as drying oils as paint vehicles with and for pigments of the metal aluminate variety.
- Having now described my invention what I claim as new and desire to secure by Letters Patent is:—
1. A new pigment comprising a metal aluminate and a metal hydroxid.
  2. A new pigment comprising a metal aluminate and a like metal hydroxid.
  3. A new pigment comprising lead aluminate and a metal hydroxid.
  4. A new pigment comprising lead aluminate and lead hydroxid.
  5. A paint comprising a metal aluminate, a metal hydroxid and a vehicle.
  6. A paint comprising a metal aluminate, a like metal hydroxid, and a vehicle.
  7. A paint comprising lead aluminate, a metal hydroxid, and a vehicle.
  8. A paint comprising lead aluminate, lead hydroxid, and a vehicle.
  9. A paint comprising metal aluminate, metal hydroxid, and an oil.
  10. A paint comprising metal aluminate, a like metal hydroxid, and an oil. 60
  11. A paint comprising lead aluminate, a metal hydroxid, and an oil.
  12. A paint comprising lead aluminate, lead hydroxid, and an oil.
  13. A paint comprising metal aluminate, metal hydroxid, and a drying oil. 65
  14. A paint comprising metal aluminate, a like metal hydroxid, and a drying oil.
  15. A paint comprising lead aluminate, a metal hydroxid, and a drying oil. 70
  16. A paint comprising lead aluminate, lead hydroxid, and a drying oil.
  17. A paint comprising metal aluminate, metal hydroxid, an oil, and a drier.
  18. A paint comprising metal aluminate, a like metal hydroxid, an oil and a drier. 75
  19. A paint comprising lead aluminate, a metal hydroxid, an oil, and a drier.
  20. A paint comprising lead aluminate, lead hydroxid, an oil, and a drier. 80
  21. A paint comprising metal aluminate, metal hydroxid, a drying oil, and a drier.
  22. A paint comprising metal aluminate, a like metal hydroxid, a drying oil, and a drier. 85
  23. A paint comprising lead aluminate, a metal hydroxid, a drying oil, and a drier.
  24. A paint comprising lead aluminate, lead hydroxid, a drying oil, and a drier.
  25. A paint comprising metal aluminate, metal hydroxid, an oil, and turpentine. 90
  26. A paint comprising metal aluminate, a like metal hydroxid, an oil, and turpentine.
  27. A paint comprising lead aluminate, a metal hydroxid, an oil, and turpentine. 95
  28. A paint comprising lead aluminate, lead hydroxid, an oil, and turpentine.
  29. A paint comprising metal aluminate, metal hydroxid, a drying oil, and turpentine. 100
  30. A paint comprising metal aluminate, a like metal hydroxid, a drying oil, and turpentine.
  31. A paint comprising lead aluminate, a metal hydroxid, a drying oil, and turpentine. 105
  32. A paint comprising lead aluminate, lead hydroxid, a drying oil, and turpentine. 110
- In testimony whereof I affix my signature in the presence of two witnesses.
- OSCAR WARREN PICKERING. [L.S.]
- Witnesses:
- F. L. WHISTNER,  
JAMES H. SCOTT.